

# UNITED STATES PATENT OFFICE.

JOHN T. GLEKLER, OF CLEVELAND, OHIO, ASSIGNOR TO THE CLEVELAND BRASS MANUFACTURING COMPANY, OF CLEVELAND, OHIO, A CORPORATION OF OHIO.

## HEAT-RESISTING ALLOY.

1,389,133.

Specification of Letters Patent. Patented Aug. 30, 1921.

No Drawing.

Application filed January 14, 1920. Serial No. 351 441.

To all whom it may concern:

Be it known that I, JOHN T. GLEKLER, a citizen of the United States, residing at Cleveland, in the county of Cuyahoga and State of Ohio, have invented a certain new and useful Improvement in Heat-Resisting Alloys, of which the following is a full, clear, and exact description.

The present invention relates to an alloy, 10 which due to its inherent physical and chemical properties forms a highly desirable and efficient metal for use in constructing articles which are to be used under certain conditions.

15 Among the important properties of the alloy the following may be stated:

1. The alloy will withstand repeated heating to high temperature without appreciable deterioration.

20 2. The surface of the article which is made of the alloy is not subject to scaling, nor even after repeated heating and cooling is there any warping, cracking or deformation.

25 3. The alloy is resistant to corrosion due to contact with corroding substances or fumes such as corrosive liquids or solids or oxidizing gases.

30 4. The alloy has a high melting point so that the article which is made of the alloy may be subjected to considerable heat without in any way endangering the structure of the article due to melting or fusing.

35 5. Articles or parts of structures made from the alloy of the present invention do not grow or increase in size even after repeated heatings, that is to say, they do not increase their dimensions.

The alloy forming the subject of this invention is eminently adapted for the making 40 of containers or boxes for heat treating or carbonizing purposes, saggars, furnace parts, crucibles, glass molds, metal molds for foundry use, retorts, dies, die rings,—in fact, any structure where the important properties of the alloy may be utilized. The alloy 45 also may be utilized for the manufacture of electrical resistance elements.

The alloy consists essentially of a combination of chromium, nickel and iron, al- 50 though there will usually appear in the final alloy some silicon and some manganese, and perchance a trace of titanium.

As is very well known, silicon and titanium are commonly used and added to a 55 bath of molten metal for deoxidizing and

scavenging purposes, and in the present instance their use is limited to this feature, but small amounts of the metals mentioned may be found in the final alloy due to the desire to insure the presence of sufficient silicon and titanium to accomplish the purposes desired.

The manganese is added to the molten metal for the purpose of giving a good grain to the alloy, and also for the purpose of preventing the formation of graphitic carbon, the manganese tending to cause the carbon present to appear in the final alloy as carbide of iron and chromium.

The alloy contains 15 to 40 per cent. of 70 chromium, 1 to 15 per cent. of nickel, with the balance consisting substantially of iron, except as before noted, the presence of slight amounts of silicon and from  $\frac{1}{2}$  of 1 per cent. to 2 per cent. of manganese.

75 The carbon in the final alloy is maintained as low as possible, preferably as low as  $\frac{1}{10}$  of a per cent. although the carbon may run as high as 2 per cent. The desirability of having the low percentage of carbon lies in 80 the fact that the final alloy is less brittle, and when the carbon is as low as 1 per cent. or under, articles made from the alloy are quite readily machined.

85 As an example of a typical analysis of an alloy found to contain the desirable qualities, the following may be given:

Chromium, 18 per cent.

Nickel, 4 per cent.

Silicon, .48 per cent.

Titanium, .2 per cent.

Manganese, 1 per cent.

Carbon, 1 per cent.

Iron, balance.

90 The chromium present imparts the highly 95 resistant qualities as to long wear and non-corrosion as well as the property of non-warping.

The nickel renders the alloy more homogeneous and less likely to crack when subjected to repeated heatings.

100 The manganese, as before stated, gives a good grain to the alloy and tends to maintain the carbon present in the final alloy in carbide form.

105 The final alloy obtained is a metal which may be easily handled in the foundry and can be cast in precisely the same manner and by the same methods as are at present commonly employed in foundry practice.

The alloy has a high tensile strength, is tough and resistant to breakage. Where the carbon present is low, the alloy is readily machined.

- 5 The alloy is preferably produced in the electric furnace by melting commercial ferrochrome together with the desired quantity of low carbon ferrous scrap material and with suitable fluxes for dephosphorizing, if 10 such a flux is necessary, and suitable fluxes for desulfurizing.

The silicon and titanium are added to the molten alloy just before pouring, and as before stated, are used for the purpose of 15 oxidizing and scavenging the metal from occluded gases.

Having described my invention, I claim:

1. An alloy which is substantially non-warping and nonoxidizing at high temperatures containing as essential ingredients 20

substantially 15 to 40 per cent. of chromium, substantially 1 to 15 per cent. of nickel, the balance consisting principally of iron.

2. An alloy which is substantially non-warping and nonoxidizing at high temperatures containing as essential ingredients substantially 15 to 40 per cent. of chromium, substantially 1 to 15 per cent. of nickel, carbon up to 2 per cent., the balance consisting principally of iron. 25

3. An alloy which is substantially non-warping and nonoxidizing at high temperatures consisting of substantially 18 per cent. of chromium, 4 per cent. of nickel, the balance consisting principally of iron and 30 carbon.

In testimony whereof I hereunto affix my signature.

JOHN T. GLEKLER.